

# UNITED STATES PATENT OFFICE

ALFRED O. BLAICH, OF CHICAGO, ILLINOIS.

## CASE-HARDENING COMPOUND.

1,138,073.

Specification of Letters Patent.

Patented May 4, 1915.

No Drawing.

Application filed October 18, 1913. Serial No. 795,873.

To all whom it may concern:

Be it known that I, ALFRED O. BLAICH, a citizen of the United States, residing at Chicago, in the county of Cook and State of Illinois, have invented new and useful Improvements in Case-Hardening Compounds, of which the following is a specification.

The purpose of this invention is to provide an improved mixture or compound for case-hardening, the basal element of which is leather.

It consists in the elements characterized and intermixed as hereinafter described as indicated in the claims.

15 Charred scrap leather constitutes the basal element employed in producing the compound which constitutes this invention. The charred leather is reduced to granular condition by any proper mechanical means 20 and intermixed with from three to five per cent. by weight of sodium salt. The two elements thoroughly intermixed constitute a very effective case-hardening compound; but especially when it is produced by the 25 method hereinafter described, which causes the leather to be impregnated with sodium salt, there is preferably comprised in the mixture about ten per cent. by weight of calcium carbonate in addition to the charred 30 leather and sodium salt.

It is sufficient for the production of a very effective compound that the elements mentioned be thoroughly intermixed mechanically, the charred scrap leather being, as stated, first reduced to granular form. But the most desirable form of the compound is produced by a process which causes the leather to be impregnated with the other 35 elements. This process is as follows:— Scrap leather is intermixed with from three 40 to five per cent. by weight of sodium salt and ten per cent. by weight of calcium car-

bonate, the three elements being thoroughly stirred together so that every granule or fragment of leather is in the immediate 45 presence of a suitable quantity of the sodium salt and calcium carbonate. The mixture is now in a liquid-sealed retort exposed to a temperature sufficient for charring the leather and for fusing the sodium salt. A 50 temperature of from 1400 to 1600 degrees F. is suitable for effecting both the charring of the leather and the fusing of the sodium salt, and the latter when fused seems to act as a vehicle for carrying the calcium carbonate into the pores of the leather, which thus becomes impregnated both with the sodium salt and the calcium carbonate, an excess of the latter usually remaining adherent to the outer surface of the leather granules or fragments, so that the three elements 55 are inseparably united; and thus there is avoided a minor defect of the product, consisting of a mere mechanical mixture of the 60 said elements, which is that they are liable to become somewhat separated by gravity in the jolting which may happen in handling 65 and transportation prior to use.

I claim:—

1. A case-hardening compound comprising 70 charred leather and a small per cent. of a sodium salt and a small per cent. of calcium carbonate thoroughly intermixed.

2. A case-hardening compound consisting 75 of charred leather impregnated by an infusion of a small per cent. of a sodium salt and a small per cent. of calcium carbonate.

In testimony whereof I have hereunto set my hand, at Chicago, Illinois, this 15th day of October, 1913.

ALFRED O. BLAICH.

Witnesses:

CHAS. S. BURTON,  
LUCY I. STONE.